

## UNITED STATES PATENT OFFICE.

WILLIAM M. DEHN, OF SEATTLE, WASHINGTON.

## PROCESS OF INCREASING THE SENSITIVENESS AND POWER OF EXPLOSIVE COMPOSITIONS AND PRODUCT THEREOF.

No Drawing.

Application filed August 20, 1920. Serial No. 404,851.

*To all whom it may concern:*

Be it known that I, WILLIAM M. DEHN, a citizen of the United States, residing in Seattle, county of King, and State of Washington, have invented certain new and useful Improvements in Processes of Increasing the Sensitiveness and Power of Explosive Compositions and Product Thereof, of which the following is a specification.

10 This invention relates to the use of diazodinitrophenol (4, 6-dinitro-2-diazophenol) as an explosive and as an ingredient in explosive compositions.

Diazodinitrophenol, the preparation of which by Peter Griess is indicated in the Annalen der Chemie und Pharmacie, 113,201; 120,126, and an improved method of manufacture whereof is disclosed by my application, Serial No. 343,592, filed Dec. 20 9, 1919, has been found by tests I have made to be highly suitable as an explosive substance and as an ingredient of explosive compositions.

Though known by Griess and others that diazodinitrophenol has explosive properties, their experiments did not reveal the fact that it possesses exceptional explosive properties, so that it has not hitherto been introduced into the explosive art.

30 Diazodinitrophenol being a diazo compound, it has apparently been assumed that it does not possess sufficient stability for commercial use as an explosive.

Such assumption is not well founded. Though detonated by spark or by percussion, diazodinitrophenol possesses sufficient stability to insure its safe manufacture, storage, and use as an explosive. Furthermore, I have found that its stability can be varied to any practical degree by mixing it either with active bases or with water and other materials.

The formula assigned to diazodinitrophenol is:



50 Though possessing the diazo structure, it may be observed that the compound possesses an exceptional diazo structure, hence possesses exceptional properties, as compared with other diazo compounds.

55 That the compound has been studied only

slightly is apparent from a view of the following description of its properties, heretofore regarded as complete. Diazodinitrophenol consists of bright yellow leaflets, slightly soluble in water, ether, benzene, 60 and alcohol. It is very soluble in acetic acid, possesses little taste and tinctorial power and is stable in cold mineral acids. It is decomposed by hot concentrated sulphuric acid, and by cold solutions of alkalies. It explodes violently when heated. Its percentage of nitrogen is 26.68. (This is a higher value than that of the respective other organic nitro compounds heretofore employed in the manufacture of explosive compositions.) 70

I have discovered the following additional properties. Diazodinitrophenol dissolves without decomposition in warm nitrobenzene and in acetone. It crystallizes as yellow transparent rectangular plates from 75 cooled nitrobenzene solutions, or from acetone solutions treated with ether or with hydrocarbon oils. It darkens in direct sunlight but is stable in diffused light. It is decomposed by many organic solvents. It 80 melts and explodes violently above 150°C. It possesses little or no noxious properties, hence differs from most organic compounds used in the explosive art.

I have found that diazodinitrophenol can 85 be stored under water at room temperatures for months without change of color and without loss of sensitiveness to explode. Furthermore, I have found that when finely divided and wet with water it cannot be exploded by a No. 8 detonating cap. Thus 90 its practical stability in handling is demonstrated. On the other hand, I have found that diazodinitrophenol, when pure and dry, can be detonated by fuse, by spark, 95 by percussion, or by friction. It can be subjected to great pressure without exploding and all compressed samples can be exploded in the different ways just mentioned. I have found that diazodinitrophenol is less 100 sensitive to shock and to friction than the fulminates and that it possesses substantially 25 to 50% more power of demolition than mercury fulminate.

Its sensitiveness to combustion and to 105 explosion, its great power of demolition, and its capacity in mixtures to increase the explosibility and brisance of the charge are its exceptional and valuable properties as an explosive.

2  
Detonating explosives themselves are comparatively rare. Detonating explosives, which on the one hand possess high power of demolition and on the other hand are inexpensive and are free from metals are practically unknown. Diazodinitrophenol answers to these qualification. Such an explosive can, therefore, be used not only as an initiator of explosions but also as a bursting charge. Furthermore it can be mixed with a great variety of explosive materials and can impart to such compositions greater sensitiveness and power of explosion. This property, to vivify and to impart brisance to common explosives, is a most valuable property of diazodinitrophenol. Especially when it is in the crystalline form and is mixed with the explosive material, without fusing, does it function in the manner described.

I have found that diazodinitrophenol in explosive compositions does not impart greater power merely by adding its own power to that of the other components of the charge, but by its capacity, as a relay of detonation, to sustain the explosive wave. For example, with 1g. charges consisting of ammonium nitrate with the indicated percentages of diazodinitrophenol and exploded by No. 6 caps, the following values were obtained in the sand bomb:

|      |     |
|------|-----|
| 0.0% | 21  |
| 0.5% | 30  |
| 1.0% | 75  |
| 5.0% | 82  |
| 60%  | 112 |
| 100% | 119 |

Without the use of diazodinitrophenol in sufficient concentration, the explosion of ammonium nitrate falls off, owing to loss of heat and owing to unfavorable conditions of moisture, density, confinement and size of crystals. With the powerful detonator diazodinitrophenol, however, the explosive wave is focally and progressively sustained, so that, for example, in the case of ammonium nitrate, with 1% of diazodinitrophenol an increase of 260% in effective power is obtained as compared with ammonium nitrate alone.

A further great advantage of diazodinitrophenol is its capacity in explosive compositions containing oxidants to utilize oxygen and thus to add to its own power. This becomes obvious in the following equations:



65 This property may be illustrated with any

of the oxidizing salts used in explosive compositions, such as the nitrates, the chlorates, and the perchlorates of the alkali metals. With potassium chloride in certain concentrations it shows greatly increased power and it is directly detonating even in concentrations less than 10%. With ammonium nitrate and ammonium perchlorate it forms smokeless combustion products. In general explosive compositions containing 25 to 100% of diazodinitrophenol are detonating.

When mixed with common oxidants, such as the oxidizing salts, or with ordinary nitro explosives, as indicated in this specification, or with the combustibles, such as wood pulp or paraffine, or with the inert materials used in explosive compositions, the sensitiveness to explode can be increased as desired, or may be held to any practical intermediate degree.

When mixed with infusorial earth, or with wood pulp, or with hydrocarbons, dynamites of varying lesser degrees of sensitiveness and power can be produced. Such dynamites, containing combustible carbonaceous material, can advantageously be mixed with active bases such as the nitrates or with nitro explosives, and thus ordinary dynamites containing small percentages of diazodinitrophenol can have increased brisance imparted thereto.

Whereas only mixtures with picric acid, trinitrotoluene, ammonium nitrate, and nitrocellulose are described in detail in this specification, I have found that diazodinitrophenol mixes as readily with the other common explosives, such as nitroglycerine, tetryl, the nitrobenzenes, and the nitronaphthalenes, and it imparts some of its characteristic properties to each of the same.

The properties referred to above make diazodinitrophenol highly suitable for use as an explosive substance by itself or in combinations with other compounds. It may be used, for example, as a filling for bombs, grenades, torpedoes, mines, and shells, as well as for the manufacture of primers and detonators, and also for all purposes for which explosive substances are used.

I have found that diazodinitrophenol alone, picric acid alone, and all mixtures of the two have substantially the same power of demolition. All mixtures of these two compounds, however, possess greater sensitiveness to explode than picric acid alone.

I have found that picric acid and diazodinitrophenol, whose melting points are 122° and above 150° respectively, can be melted in hot water when their percentages are within certain limits. For example, equal weights of the two substances melt under water yielding a product whose specific gravity is 1.75 and which detonates with fuse or with percussion. This remarkable melting property insures an easy and safe method of

blending these two explosives. The manufacture of such mixtures can therefore be effected without handling the dried and dangerous components, and the fused mixtures 5 can be drawn up into detonating fuses or can be poured directly into the shell or other containers. When desired the solidified mixtures can be pulverized under water and subsequently dried. Since all mixtures of the 10 two components possess substantially equal strength but greater sensitiveness to explode than picric acid alone, such mixtures are very useful in the art of explosives.

I have found that contact of certain percentages of picric acid and diazodinitrophenol with acetone, ethyl acetate, or with other solvents yields products, which when freed from the solvent, melt below 100°. This method of plasticising their mixtures 15 is also very useful in the art of explosives. Since all such mixtures possess greater brisance than picric acid alone, diazodinitrophenol provides a vivifying ingredient of all such mixtures, and any desired quickened combustion and brisance, within the 20 limits of brisance of the two components, can be imparted to their mixtures.

I have found that diazodinitrophenol dissolves in trinitrotoluene when the latter is 25 present in excess of 70% and the mixtures are heated at 100°, either alone or under water. The fused mixtures can either be poured into containers or can be poured into water in a thin stream, thus yielding a fine 30 powder. This powder can also be obtained safely, after cooling the melt, by grinding under water. When dried this powder is useful as a "booster" charge and as an ingredient of other explosive compositions. 35 This property can be availed of to great advantage since trinitrotoluene alone is often too insensitive toward detonating charges. Substantially any desired sensitiveness to 40 explode can be obtained by blending trinitrotoluene with diazodinitrophenol. Furthermore all such mixtures possess greater strength than trinitrotoluene itself.

I have found that diazodinitrophenol and 45 nitrocellulose can be blended by the solvent effects of acetone and by other organic solvents and that, when freed from such solvents, the mixtures are more or less plastic, yellow, colloidal masses possessing greater sensitiveness and power than the nitrocellulose alone. These mixtures are useful in the 55 art of explosives.

I have found, as indicated above, that diazodinitrophenol can advantageously be mixed with ammonium nitrate to form powders which can be used for a variety of purposes, since they are smokeless and powerful 60 and can be made to detonate. When the percentages of diazodinitrophenol in these powders is substantially less than 50%, oxygen 65 available for combustibles or for nitro ex-

plosives is supplied by the ammonium nitrate. A great variety of such explosive compositions, all within the scope of my claims, can be prepared. Some of these are shown in the following table. The measurements of power were all made on 1g. charges exploded by No. 6 caps in the sand bomb; the values given are grams of 20-30 mesh sand crushed.

75

| Materials.           | A     | B     | C     | D     | E     | F     | G     | H     | I     | J     | K     |
|----------------------|-------|-------|-------|-------|-------|-------|-------|-------|-------|-------|-------|
| Diazodinitrophenol   | 5     | 5     | 5     | 5     | 50    | 5     | 2     | 5     | 5     | 5     | 72    |
| Ammonium nitrate     | 54    | ..... | 63    | ..... | ..... | 90    | 80    | 80    | 95    | 28    | 80    |
| Trinitrotoluene      | 41    | 95    | ..... | ..... | ..... | ..... | ..... | ..... | ..... | ..... | ..... |
| Dinitrobenzene       | ..... | 95    | 32    | ..... | 50    | 95    | 8     | ..... | ..... | ..... | ..... |
| Picric acid          | ..... | ..... | ..... | ..... | 100   | ..... | ..... | ..... | ..... | ..... | ..... |
| Wood pulp            | ..... | ..... | ..... | ..... | ..... | ..... | 15    | ..... | ..... | ..... | ..... |
| Starch               | ..... | ..... | ..... | ..... | ..... | ..... | ..... | 15    | ..... | ..... | ..... |
| Relative power       | 100   | 62    | 91    | 95    | 121   | 116   | 78    | 98    | 86    | 82    | 123   |
| Power without DDP    | 80    | 57    | 64    | 59    | 115   | 115   | ..... | 66    | 51    | 22    | ..... |
| % increased with DDP | 25    | 9     | 42    | 7     | 5     | 1     | ..... | 48    | 70    | 272   | ..... |

85

It will be observed that in general percentages of increase of power are greater than the percentages of diazodinitrophenol used; and further, these mixtures containing diazodinitrophenol are more easily ignited and exploded by impact than the corresponding compositions without the diazo- 90 dinitrophenol.

95

My process, involving as it does a powerful distributive booster charge, reveals further advantages in that it admits of compression to greater densities, it admits of the presence of greater percentages of adventitious water or other inert material, it overcomes deficiencies in confinement, and it dispenses with special contrivances for 100 ordinary booster charges.

105

I claim:

1. The process of increasing the sensitiveness and power of explosive compositions which comprises mixing diazodinitrophenol and other explosive matter under water and subsequently drying, substantially as described.

110

2. The process of increasing the sensitiveness and power of explosive compositions which comprises mixing diazodinitrophenol with other explosive material and inert material under water together and subsequently drying, substantially as described.

115

3. The process of increasing the sensitiveness and power of explosive compositions which comprises fusing nitro explosives and diazodinitrophenol under water and subsequently freeing the mixture from water, substantially as described.

120

4. The process of increasing the sensitiveness and power of explosive compositions which comprises incorporating with said explosive material a smaller proportion of diazodinitrophenol moistened with water to 130

- render it safe during incorporation therewith.
5. The process of increasing the sensitivity and power of explosive compositions which comprises incorporating with said explosive material a lesser proportion of diazodinitrophenol in the presence of water and subsequently freeing the mixture from water, substantially as described.
- 10 6. An explosive material comprising diazodinitrophenol together with other explosive material.
7. An explosive comprising diazodinitrophenol together with ammonium nitrate.
- 15 8. An explosive comprising diazodinitrophenol together with other explosive material and inert material.
9. An explosive comprising diazodinitrophenol together with ammonium nitrate and inert material.
10. An explosive comprising diazodinitrophenol together with other explosive material and oxidant material.
11. An explosive comprising diazodinitrophenol together with other explosive material, oxidant material, and inert material.

In witness whereof, I have signed my name hereto.

WILLIAM M. DEHN.